

F. J. METZGER.

FURNACE REACTION CHAMBER AND METHOD OF PREVENTING DESTRUCTION THEREOF.  
APPLICATION FILED FEB. 6, 1920.

1,363,428.

Patented Dec. 28, 1920.

Fig. 1,



Fig. 2,



Floyd J. Metzger Inventor  
By his Attorneys  
Emmie Davis Meuron & Edmunds

# UNITED STATES PATENT OFFICE.

FLOYD J. METZGER, OF NEW YORK, N. Y., ASSIGNOR TO AIR REDUCTION COMPANY, INC., A CORPORATION OF NEW YORK.

## FURNACE REACTION-CHAMBER AND METHOD OF PREVENTING DESTRUCTION THEREOF.

1,363,428.

Specification of Letters Patent. Patented Dec. 28, 1920.

Application filed February 6, 1920. Serial No. 358,733.

To all whom it may concern:

Be it known that I, FLOYD J. METZGER, a citizen of the United States, residing at New York, in the county of New York, State of New York, have invented certain new and useful Improvements in Furnace Reaction-Chambers and Methods of Preventing Destruction Thereof; and I do hereby declare the following to be a full, clear, and exact 10 description of the invention, such as will enable others skilled in the art to which it appertains to make and use the same.

This invention relates to furnace reaction chambers used, for example, in the fixation 15 of nitrogen, more particularly by methods involving the heating of mixtures of alkali metal compounds and carbon with nitrogen in the presence of a catalytic agent such as iron, whereby a furnace product containing 20 alkali metal cyanid is obtained. Such a method as described in U. S. Patent No. 1,322,195, has been successfully operated by employing mixtures of alkali metal carbonate or oxid with coke and iron, the mix- 25 ture being heated while nitrogen or nitrogenous gases pass through the reaction chamber.

Reaction chambers of the character de- 30 scribed are subjected to direct contact with combustion gases which, being of an oxidizing character rapidly destroy iron or steel at the relatively high temperatures em- 35 ployed. It has been found desirable, there- fore, to construct such chambers of a rela- tively resistant material such as nichrome, 40 an alloy of nickel and chromium containing substantially 57% of nickel and 14% of chromium with 27% of iron and 2% of man- gane. Nichrome reaction chambers in the 45 form of tubes, are generally cast and are subject to sand holes and pores, which some- times extend through the tube wall. In the 50 practice of the method, the alkali metal car- bonate, which does not combine directly with the metal, works through these sand 55 holes to the exterior and there combines with the surface film of oxid, produced by oxygen in the highly heated combustion gases em- 60 ployed in maintaining the required tempera- ture. The result of the contact of alkali 65 metal carbonate with the metallic oxid is the formation of a blister which gradually 70 works back through the tube until a hole 75 is formed which ruins the apparatus. As

nichrome tubes are relatively expensive, the loss entailed is a material factor in the cost of producing cyanid.

The object of the present invention is to overcome the disadvantages resulting from the use of cast nichrome tubes and I have 60 discovered a simple remedy which entirely obviates the difficulty by closing the sand holes or other minute pores, through which the alkali metal carbonate may work its way to the exterior of the tube. 65

I have been enabled to accomplish the de- 70 sired result applying a plating of nickel to the interior of the tube and thereby closing the sand holes and pores in the metal. The nickel may be applied electrolytically in an 75 expeditious and satisfactory manner and when the tube is thus internally coated, it may be used continuously for long periods without danger from the destructive action of the alkali metal carbonate as hereinbefore 80 described.

In the accompanying drawing, I have 85 shown one form of my invention in Figure 1, in section together with an illustration in Fig. 2 of the destructive action to which the 90 tube is otherwise subjected.

Referring to Fig. 2 the tube 5 is shown in section with a sand hole 6, which is, of course, greatly magnified, extending through the wall. At the exterior of the tube the 85 blister 7 is shown, eating its way through the tube as the alkali metal carbonate gradually combines with oxid on the surfaces at the bottom of the blister. Eventually the 90 blister will extend through the wall of the tube which is then worthless.

In Fig. 1, the tube 8 is shown in section with a coating 9 of nickel deposited on its internal surface. The coating 9 is homo- 95 geneous and continuous, it being a com- paratively simple matter to obtain such a coating by electroplating. All of the minute sand holes and pores 11, which might other- wise provide outlets for the alkali metal carbonate, are thus closed and the action 100 illustrated in Fig. 2 is thereby prevented.

Obviously the preservation of the expen- 105 sive nichrome tubes is of great advantage in the practice of the nitrogen fixation method as described; and I desire, therefore, to claim my invention broadly as involving the application of a thin continuous metal coating to the interior of tubes employed as

reaction chambers in the practice of such methods.

Various changes may be made in the details of construction of the tube and in the mode of applying the coating without departing from the invention or sacrificing any of its advantages.

I claim:

1. A reaction chamber for high temperature methods in which the chamber is externally heated by oxidizing gases and employing a substance which is adapted to combine with the oxid formed on the outer surface of the chamber, said chamber having a wall of nichrome and an internal coating of a resistant metal applied to the inner surface of said wall and closing the pores therein.
2. A reaction chamber for high temperature methods in which the chamber is externally heated by oxidizing gases and employing a substance which is adapted to combine with the oxid formed on the outer surface of said chamber, said chamber having a wall of nichrome and an internal coating of nickel applied to the inner surface of said wall and closing the pores therein.
3. A reaction chamber for high tempera-

ture methods in which the chamber is externally heated by oxidizing gases and employing a substance which is adapted to combine with the oxid formed on the outer surface of said chamber, said chamber comprising a tube of cast nichrome having a coating of nickel applied to its inner surface.

4. A method of preventing destruction of nichrome tubes employed in carrying out high temperature reactions by externally applied heating gases and with a substance which is adapted to combine with the oxid formed on the outer surface of said chamber, said method comprising the application of a coating of a resistant metal to the inside of said tube.

5. A method of preventing destruction of nichrome tubes employed in carrying out high temperature reactions by externally applied heating gases and with a substance which is adapted to combine with the oxid formed on the outer surface of said tube, said method comprising the application of a coating of nickel to the inside of said tube.

In testimony whereof I affix my signature.

FLOYD J. METZGER.